

Dec. 18, 1928.

1,695,595

W. A. LARNED

ELASTIC METAL STRINGING AND METHOD OF MAKING THE SAME

Filed July 12, 1923

2 Sheets-Sheet 1



FIG. 2



FIG. 4



FIG. 6



FIG. 3



FIG. 1

INVENTOR,  
William A. Larned  
BY  
Howard S. Smith,  
His ATTORNEY.

Dec. 18, 1928.

W. A. LARNED

1,695,595

ELASTIC METAL STRINGING AND METHOD OF MAKING THE SAME

Filed July 12, 1923

2 Sheets-Sheet 2



FIG. 5

INVENTOR,  
*William A. Larned*  
BY  
*Howard S. Smith*  
*His ATTORNEY*

Patented Dec. 18, 1928.

1,695,595

# UNITED STATES PATENT OFFICE.

WILLIAM A. LARNED, OF SUMMIT, NEW JERSEY, ASSIGNOR TO THE DAYTON STEEL RACQUET COMPANY, OF DAYTON, OHIO, A CORPORATION OF OHIO.

## ELASTIC METAL STRINGING AND METHOD OF MAKING THE SAME.

Application filed July 12, 1923. Serial No. 651,036.

My invention relates to new and useful improvements in an elastic metal stringing, and the method of making the same, and has particular reference to a nine-wire stringing 5 that is preferably made up of three groups of three wires each, for tennis rackets and the like.

It is the principal object of my invention to provide an elastic metal stringing which is 10 made up of wires that are first wound into groups, after which the groups themselves are wound together and then stretched to a blocking point, or a point beyond which the stringing has a maintained elasticity due to 15 the torsional reaction of the groups upon each other.

In constructing this stringing I preferably employ three groups of three wires each, since it has been found that a nine-wire 20 stringing so made up more nearly approaches the characteristics of gut without its disadvantages. In other words, such a stringing gives all the advantages of a gut stringing in that it has a large amount of elasticity and a 25 small amount of set, without the attendant disadvantages of gut under dampness.

In the accompanying drawings illustrating my invention, Figure 1 is a perspective view of three wires that are wound together in a 30 group, the winding being incomplete at one end to show the wires themselves. Figure 2 is a cross sectional view taken through said group on the line 2—2 of Figure 1. Figure 3 is a perspective view of three groups of 35 three wires each, showing how the groups are loosely wound together before being stretched to the blocking point for insertion in a tennis racket frame. Figure 4 is a cross sectional view taken through the same on the line 4—4 of Figure 3. Figure 5 is a plan 40 view of a tennis racket containing my nine-wire stringing after it has been stretched to the blocking point. And Figure 6 is a cross sectional view of the stringing after it has 45 been inserted in the tennis racket frame, taken on the line 6—6 of Figure 5.

Throughout the specification and drawings, similar reference characters denote corresponding parts.

Referring to the accompanying drawings 50 for a detailed description of my improved stringing, the numerals 1, 2 and 3 in Figure 1 designate three wires that are preferably of the best grade of steel and of uniform length 55 and diameter. These wires are preferably

wound together left-handed, without a core, to form a group 4.

Three of the groups 4 are then wound in the opposite direction, or right-handed in this instance, around a core to form a larger 60 group 5. The core is then removed to leave the wires loosely wound about a hollow center as shown in Figures 3 and 4. The group 5 is then stretched to a blocking point, or a point beyond which it will have a maintained 65 elasticity under the impacts of a tennis ball after it is inserted in a tennis racket frame 6.

Tests which have been made with an Olsen testing machine show that under a blow of 60 pounds, which represents approximately 70 the force with which the ball is hit by an average tennis player, my grouped nine-strand stringing will give better results than gut. Under such a blow the tests showed that the grouped nine-strand stringing had 75 an elasticity of 8% and an elongation of 1.7% as compared with an elasticity of 6.6% and an elongation of 2.1% for the gut stringing under the impact of the same force. Under a blow of 70 pounds, which represents 80 substantially the force with which the ball is struck by an exceptional player, the grouped nine-strand stringing had an elasticity of 7.3% and an elongation of 2.8%, and the gut stringing an elasticity of 8.1% and an elongation 85 of 2.6%.

The above tests show that my grouped nine-wire stringing has all the advantages of gut in the way of a large amount of elasticity and a small amount of elongation or set. Reduction in elongation prevents the racket stringing from becoming soft or loosening up. Like gut, my grouped nine-wire stringing also presents a rough or ridged surface to the ball so that it may take a firm grip 95 upon the latter in play.

While possessing all the advantages of gut, my nine-strand stringing has none of its disadvantages, for it will not deteriorate in hot or damp weather as gut will do.

Having described my invention, I claim:

1. An elastic metal stringing comprising groups of wires that are first wound together in a loose state, and then stretched to a point beyond which they will torsionally engage 105 each other to provide maintained elasticity under the action of a force.

2. The method of making an elastic metal stringing, which consists, first, in winding individual wires into groups, then winding 110

the latter into a larger group, and then stretching the latter to a point beyond which the individual groups comprising it will torsionally engage each other to give maintained elasticity under the action of a force.

3. The method of making an elastic metal stringing, which consists, first, in winding individual wires into groups, then winding the latter around a core into a larger group, then removing the core and stretching the larger group to a point beyond which the individual groups comprising it will torsionally engage each other to give maintained elasticity under the action of a force.

4. The method of making an elastic metal <sup>15</sup> stringing, which consists, first, in winding individual wires in one direction into groups of three, then winding three of said groups in the opposite direction to form a larger group, and then stretching the latter to a <sup>20</sup> point beyond which the individual groups comprising it will torsionally engage each other to give maintained elasticity under the action of a force.

In testimony whereof I have hereunto set <sup>25</sup> my hand this 5th day of July, 1923.

WILLIAM A. LARNED.